

Aug. 10, 1926.

1,595,312

W. G. O'BRIEN

FOOTWEAR

Filed July 31, 1922



FIG. 3



FIG. 1



FIG. 4



FIG. 2

INVENTOR

BY WILLIAM G. O'BRIEN  
R. A. Wagner,  
his ATTORNEY

U.S. Patent

Patented Aug. 10, 1926.

1,595,312

# UNITED STATES PATENT OFFICE.

WILLIAM G. O'BRIEN, OF AKRON, OHIO, ASSIGNOR TO THE GOODYEAR TIRE & RUBBER COMPANY, OF AKRON, OHIO, A CORPORATION OF OHIO.

## FOOTWEAR.

Application filed July 31, 1922. Serial No. 578,744.

My invention relates to foot-wear and it has particular relation to a substitute for the commonly used leather shoe. The object of my invention is to provide a material 5 which is both porous and water-resistant, which may be molded to the desired shape and size, and which shall be particularly adaptable for the construction of both the uppers for shoes and for entirely unitary 10 shoes.

Heretofore it has been customary to make shoes either entirely of leather, or with the upper portion thereof composed of leather. Certain leather substitutes have been 15 experimented with, particularly for soles. Generally speaking, these substitutes were objectionable because of the fact that they were non-porous. The success of leather as a material for constructing shoes results 20 principally from the fact that it is porous but water-resistant, which permits of the evaporation of perspiration from the foot of the wearer, but prevents the admission of moisture thereto. Those substitutes for 25 leather which have been proposed, heretofore, have not been porous, thus preventing the evaporation of perspiration from the foot and rendering the wearer uncomfortable, as well as producing an unhealthy condition of 30 the foot.

By my invention I have obviated the aforementioned objection by providing a tough, flexible, water-resistant material of 35 good wearing qualities which is porous and which can be made to resemble leather to such degree that even an expert cannot determine with certainty whether or not it is leather.

In the accompanying drawings:

40 Fig. 1 is a view in side elevation of a molding machine, which operates on the principle of the Drake process, adapted for the construction of shoes;

45 Fig. 2 is a similar view of a machine adapted for the construction of shoe uppers only;

50 Fig. 3 is a very much enlarged view of the material which I employ in constructing shoes; and

55 Fig. 4 is an elevational view of a screen adapted to produce a flat piece of material of a predetermined size and shape.

In practicing my invention I have found that the best results may be obtained in the following manner. A quantity of fibers,

which may be of wood, hemp, jute, leather, wool, cotton, asbestos, or the like, is thoroughly beaten, usually in a beater of the Holland type, so as to separate the various fibers thereof. The fibers are then removed from 60 the liquid in which they are beaten and if beaten in water, this must be removed either by displacement with alcohol or with a mixture of alcohol and water. The fibers are then thoroughly dispersed in a quantity of 65 liquid composed of approximately 77% toluol and 23% alcohol. While I have referred to the liquid as being composed of a mixture of toluol and alcohol, it might equally well be composed of benzol and acetone, 70 the essential feature being that the liquids be miscible and that one be a solvent of rubber and the other a precipitant thereof.

A quantity of rubber, dissolved in toluol, is then added to the mixture and thoroughly 75 dispersed therein. The best results will ordinarily be obtained by having the quantity of rubber and that of fiber approximately equal in weight, and each equal to from  $\frac{1}{2}$  to 2% of the weight of the combined liquids. The solution is then so treated as to bring about precipitation of the rubber on the fibers. This may be accomplished either by the addition of alcohol, or some other suitable precipitating agent, to the mixture, 85 or by reducing the temperature of the mixture to a suitable point.

The liquid, having the rubber coated fibers suspended therein, may now be treated in any one of several different ways to secure 90 the desired final result. It may be placed in a pulp molding machine of the Drake type, disclosed in Patent No. 1,305,203, and as illustrated in Fig. 1 of the drawings. In this figure the screen mold conforms to the 95 shape of the shoe which it is desired to build, or it may conform only to the shape of the shoe upper, as illustrated in Fig. 2. By means of compressed air, suitably directed, the fibers are arranged in a matted formation 100 in the desired shape and steam is then employed for drying and curing the rubber. If desired, the compressed air may be heated, thus combining the drying and curing operations. The thickness of any portion of 105 the shoe, or of the upper, may be regulated by properly controlling the compressed air entering the mold, as described more fully in the Drake patent referred to above.

Referring to the accompanying drawing 110

for a more detailed description of my invention, a tank 4 is provided with a downwardly extending portion 5, which is provided with a hose connection 6 and a valve mechanism 7. The lower end of the portion 5 of the member 4 is provided with an extension 8 in the form of a pipe, the lower end of which is externally threaded. The member 5 is also provided with a flange 9 which 10 serves to support a screen mold 10, of any desired configuration. In Fig. 1 the screen mold conforms to the shape of an entire shoe. In threaded engagement with the lower end of the portion 8 is a member 11, which may be adjusted vertically so as to 15 permit of regulation of the air pressure striking the bottom of the shoe.

The container 4 is normally filled with the pulp from which it is desired to make 20 the shoe. Upon opening the valve 7, a quantity of the pulp descends through the portions 5 and 8 to the bottom of the screen mold 10. The valve 7 is then closed and compressed air is admitted to the member 25 8 by means of the air connection 6. By suitably controlling the pressure of the air, the distribution of the pulp may be regulated at will, particularly as to thickness, as described more fully in the Drake patent 30 previously mentioned. The pulp is spread, by means of the compressed air, into a layer of any desired thickness which covers the inside of the screen 10. After the pulp has been suitably distributed by 35 the compressed air, heated air is admitted through the connection 6, which dries the product while it is still attached to the mold 10. The rubber is then cured by any suitable method.

40 The mold must be so made as to be readily opened to remove the shoe form. This will usually be performed by having the two halves of the screen hinged together at one side and adapted to separate along the remaining edges.

In Fig. 2 I show a structure very similar to that shown in Fig. 1 except that the pressure adjusting member 11 is replaced by an adjusting member 12 of a shape 50 corresponding to some extent, to that of the shoe, which it is believed will aid in the proper distribution of the pulp therein. Also, the bottom of the screen is provided with a solid member 13 which prevents the deposition of pulp thereon since air cannot 55 pass therethrough. The structure shown in Fig. 2 is adapted for the formation of a shoe upper only, whereas that shown in Fig. 1 is adapted for the construction of 60 the entire shoe.

Fig. 3 is a view representing, as nearly as it can be drawn, the material which I employ for making shoes. It will be noted from this figure that the various rubber 65 coated fibers become thoroughly intertwined

and tangled when permitted to assume their natural positions, which provides a composition of considerable strength. By the use of fibers interlocked and attached together as described, a porous but water-resistant 70 flexible composition is provided. The size of the individual fibers depends upon the size of the original fibers placed in the solution, and on the amount of rubber deposited thereon. The dimensions of the interstices 75 between the fibers depend to a large extent upon the pressure by which the material has been compressed during manufacture. The interstices between the fibers are indicated quite clearly in Fig. 3.

80 Another method of treating the fibers after they have been coated with rubber and are still in suspension in the liquid, consists of screening them from the liquid through a flat or otherwise suitably shaped 85 screen, as illustrated in Fig. 4 of the drawings in such manner as to provide a uniformly thick matted formation. In Fig. 4 is illustrated a screen 14 mounted upon a skeleton framework 15 and of the exact contour 90 of the upper of a shoe. The screen 14 is flat and when properly operated produces a mat of the desired size and shape, thus eliminating the waste incident to cutting irregularly shaped designs from flat 95 sheets of material. When this method is employed, it is highly desirable that the quantity of fibers be very small compared to the total quantity of the liquids in which they are suspended, so that when strained 100 therefrom, the fibers may assume their natural position with respect to each other, which provides a very good matted formation. The mat formed on the screen is washed, and cured in the usual manner.

105 From the foregoing description, it will be apparent that I have provided a method of forming a leather substitute which will perform all of the functions of leather, and which may be made of any desired shape and thickness. This eliminates the waste which necessarily occurs when material, such as leather which naturally occurs in sheets, is cut up for the purpose of constructing shoes. It will also be apparent that when the rubber coated fibers are permitted to seek their natural position, either by being carefully strained from a liquid, or by being deposited 110 on the screen by means of compressed air, that numerous minute interstices will occur 115 between the fibers, the size and number of which depends upon the method of finishing the material. When properly formed, these openings are of such dimensions that liquid 120 cannot readily pass therethrough, but the material permits diffusion of gas and air.

125 Generally, I have found it advisable to give the composition a wax finish, which improves the appearance thereof and increases the surface tension of any water which may 130

be deposited thereon, thereby aiding in rendering the composition water-resistant. The wax finish also improves the appearance of the product.

- 5 Although I have described several forms of my invention and one application thereof, it will be obvious to those skilled in the art that it is not so limited but that various minor modifications and changes 10 may be made therein without departing from the spirit of my invention, or from the scope of the appended claims.

What I claim is:

- 15 1. A molded shoe upper composed of a porous water-resistant synthetic composition of uninterrupted texture of fiber and rubber.
2. A molded shoe upper composed of a porous water-resistant material of uninterrupted

texture including rubber coated fibers uniformly distributed in matted relationship.

3. An article of manufacture comprising a molded shoe composed of a porous water-resistant material of uninterrupted texture including rubber having fibers dispersed 25 therein intertwined with each other provided with a wax finish.

4. A molded shoe comprising a water-resistant body portion of rubber coated uniformly distributed matted fibers, porous to 30 air and vapor and of uniform thickness throughout.

In witness whereof, I have hereunto signed my name.

WILLIAM G. O'BRIEN.